

## UNITED STATES PATENT OFFICE

2,398,986

## PHOTOGRAPHIC COMPOUND

Woodrow Othell Wilson, Los Angeles, Calif., assignor to Wilson Lorraine Company, Los Angeles, Calif., a partnership composed of Woodrow Othell Wilson and Louis J. Platt

No Drawing. Application February 1, 1944,  
Serial No. 520,695

2 Claims. (Cl. 95—6)

This invention relates to the art of photography and deals particularly with a light sensitive substance suitable for making negatives, prints, and the like.

The invention to be described hereinafter has been developed primarily for use in the blueprint field, but as the description proceeds it will become evident to those skilled in the art that the above mentioned substance also referred to herein as a photographic compound will have usefulness in any field where a light sensitive material may be used.

The primary object of this invention is to provide a photographic compound characterized by speed in response to light exposure, permanence in reproduction, ease of application for use, convenience and economy in preparation, and inexpensive ingredients which go to make up the compound. The light sensitive material to be disclosed herein has been found in practice to have a very high light speed; that is, the time of exposure of my compound is very short when compared with the time required by the average blueprint compound used today. It has been found that, generally stated, the speed of exposure of my compound may be in the neighborhood of forty-five seconds. Also, tests have been made which prove that reproductions made with my compound do not appreciably fade over a period of several years. In addition, the light sensitive material may be applied to the base or matrix upon which the reproduction is to be made, either by hand or machine, and may be done a short while before the exposure is made. Furthermore, the ingredients in the compound are common inexpensive chemicals and may be mixed in the ordinary manner without resorting to a dark room. Other objects and advantages will appear as the description proceeds.

Briefly stated, my invention consists in a new combination of chemicals which react to produce a light sensitive substance. As before stated, the substance is highly sensitive to light and will yield upon exposure a gradation in intensity comparable to the exposure.

The compound comprises ferrous ammonium citrate, potassium ferricyanide, and potassium bichromate, mixed in the following manner and in the following proportions.

First: Dissolve one hundred grains of ferrous ammonium citrate in one ounce of distilled water.

Second: Dissolve fifty grains of potassium ferricyanide in one ounce of distilled water.

Third: Mix the two solutions together, forming two ounces of solution.

Fourth: Dissolve one grain of potassium bichromate in the solution from the above steps.

Fifth: Filter the solution and it is ready for use.

It is to be understood that the above amounts may be made more or less as desired, the only limitation being that the proportions remain the same; also, steps one and two may be reversed in order but step four should not be changed in its sequence.

15 The solution is applied as a light sensitive covering to papers, metal surfaces, textiles, or any other substance desired by either spraying it on or painting it on with a suitable brush. Materials sensitized in this manner may be exposed in the 20 ordinary way and the reproductions developed in a water bath. The color of the reproductions normally are blue, and various shades of blue may be obtained by regulating the exposures, the intensity of the color being directly proportional to 25 the exposure. The reproductions are substantially permanent and may be subsequently treated in any well known manner for bleaching, or to obtain different colors, etc.

30 Having set forth my invention in general terms, what I claim as new and patentable is:

1. A photographic compound consisting essentially of two parts of ferrous ammonium citrate and one part of potassium ferricyanide dissolved 35 in water with one fiftieth ( $1/50$ ) part of potassium bichromate dissolved therein.

2. The method of making a photographic compound consisting in mixing the following ingredients in their following respective proportions: one hundred (100) grains of ferrous ammonium citrate dissolved in one ounce of water, fifty (50) grains of potassium ferricyanide dissolved in one ounce of water, combining the two solutions and dissolving therein one (1) grain of 45 potassium bichromate.

WOODROW OTHELL WILSON.